

Jan. 22, 1946.

D. M. MUSSER ET AL

2,393,553

PROCESS OF PULP PREPARATION AND PRODUCT THEREOF

Filed Dec. 5, 1940



INVENTORS

David M. Musser  
Harry C. Engel  
Mason & Porter  
ATTORNEYS

## UNITED STATES PATENT OFFICE

2,393,553

PROCESS OF PULP PREPARATION AND  
PRODUCT THEREOF

David M. Musser and Harry C. Engel, Pittsburgh,  
Pa., assignors, by mesne assignments, to Na-  
tional Cotton Council of America, Memphis,  
Tenn., a corporation of Tennessee

Application December 5, 1940, Serial No. 368,730

5 Claims. (Cl. 92—21)

This invention relates to the art of preparing cellulose pulps, for the purpose of decreasing the beating time and increasing the quality of the products formed.

When it is sought to utilize raw cotton fibers, or cotton fibers which have been purified under mild kiering and bleaching conditions, for paper manufacture, the procedure is hindered to a large extent by the lack of satisfactory methods to process these fibers properly for converting them into fibers of desired properties. It is well known that cotton fibers resist heating and undergo fibrillation with great difficulty. A comparatively long beating period is therefore necessary to reduce them to suitable fineness for paper stock. This long beating time is expensive and tends to slow down mill operations; and has the serious defect that it extensively impairs the utility of the fibers by causing transverse breaking of these fibers prior to the splitting incident to fibrillation. Consequently, the resultant paper product possesses poor folding and mechanical properties, as compared with a wood pulp or rag stock that is more easily hydrated.

It has previously been sought to decrease the beating time for such cotton fibers through the use of acidic or oxidizing agents or conditions, but fundamental success has not been encountered because the treatments are difficult to control and generally are so drastic that the fibers are seriously impaired as an incident to reducing them to the condition at which beating can proceed. That is, such treated cellulosic fibers are permanently damaged, and the paper products are of inferior quality.

Upon investigation, it has been found that cellulosic pulps can be obtained in the manner hereinafter described in order to yield a paper stock superior to those made according to prior art. In particular, it has been found that if the cellulosic pulp is beaten in the presence of a small amount of water-soluble cellulose derivative, such as methyl cellulose or ethyl cellulose, the beating time is definitely decreased and the paper-making properties of the resulting stock are greatly improved over those obtained by prior processes.

According to the invention, therefore, a material is introduced during the beating period for producing a more rapid fibrillation per unit of beating time, and being further effective for yielding a paper stock superior to the stocks beaten for a normal or longer period.

In practicing the invention, the treating agent is introduced to the charged beater at the start of the beating process. This agent is introduced

preferably in the form of a solution or dispersion in water, but may be employed in a dry or powdery form where a proper condition of beating is established to assure the distribution and operation of the material during the course of the beating period. Thus, if the beating period is less than 2 hours, the best results appear to be obtained if, for example, methyl cellulose is added in the form of a solution; while if the beating period is greater than 2 hours, the methyl cellulose may be introduced in powder form. In these two illustrative cases, no significant difference in properties of the paper sheets was observed between the conditions of adding the methyl cellulose as a solid or as a solution. It will be understood that herein the methyl or ethyl cellulose is referred to as water-soluble for the reason that it swells and disperses in the presence of pure water to form a liquor which has the commonly accepted attributes of a solution.

As an illustration of the extent to which the beating time may be decreased, a bleached kraft pulp was subjected to a beating operation in a commercial beater for periods of 1½ hours, in 25 comparison runs where one run included the employment of 6.0 percent of methyl cellulose (based on the weight of dry pulp, and used as a 0.3% solution), while the companion run omitted the methyl cellulose. The result of such runs is as 30 follows:

TABLE I  
Data on kraft pulp

|    |                                | Run No. |       |       |       |       |
|----|--------------------------------|---------|-------|-------|-------|-------|
|    |                                | 17      | 18    | 19    | 20    | 21    |
| 35 | Beating..... hours.            | 0.5     | 0.5   | 1.0   | 1.5   | 1.5   |
|    | Methyl cellulose..... percent. | 0       | 6.0   | 0     | 0     | 6.0   |
| 40 | Tear.....                      | 128     | 102   | 111.0 | 86    | 74.0  |
|    | Breaking length.....           | 4,430   | 6,270 | 5,130 | 6,260 | 7,580 |
|    | Burst.....                     | 40.8    | 58.2  | 43.7  | 57.4  | 73.6  |

In these tabulations, the TAPPI standard tests were employed. The "breaking length" is the length of a strip of paper, cut either in machine or cross direction, which would break of its own weight when suspended vertically; and is a value calculated from the tensile strength and basis weight of a sheet and is expressed in meters. Bursting strength is measured by the pressure required to rupture a specimen when tested under the specified conditions; and the burst factor or "burst" is the numerical value obtained by dividing the bursting strength in grams per square centimeter by the basis weight of the sheet in

grams per square meter. Tearing strength is measured by the force required to tear a specimen under standardized conditions in an instrument designed to simulate in a general way the tearing encountered under use conditions: the tearing factor or "tear" is the tearing strength in grams per sheet divided by the basis weight in grams per square meter.

From this Table I, it will be noted that the breaking length and burst value increase relatively greatly with methyl cellulose for each interval of beating time, while the tear value decreases: this indicates that the methyl cellulose is expediting the beating process. Thus, by comparing runs 18 and 20, it will be noted that the breaking length after one half hour of beating, with 6.0 percent of methyl cellulose, is equivalent to the value obtained by beating for 1½ hours without methyl cellulose, and that a corresponding burst value likewise results. On the other hand, it will also be noted from runs 18 and 20 that the tear value is higher in the methyl cellulose run, as might be expected from the shorter beating time utilized.

It has further been found that the concentration and viscosity of the treating material play important roles. For example, it has been found that the high and extra high viscosity types of methyl cellulose are more effective than the low and medium viscosity types. That is, for a given weight of methyl cellulose, the high viscosity type expedites beating and enhances the physical properties of the paper to a greater extent than the same weight of the low viscosity type. In making these comparisons, the viscosities of the methyl cellulose were based upon the time required for a definite volume of a 2 percent aqueous solution at 20 degrees C. to flow through a standardized Ubbelohde capillary tube. A low viscosity type runs from 20 to 30 centipoises, with an average at 25; a medium type between 40 and 60, with an average at 50; a high viscosity type at 80 to 120, with an average at 100; and an extra high viscosity type between 250 and 350, with an average at 300.

This appears from the following tabulation of results obtained by beating hull fiber pulp for 7 hours with 6.0 percent of methyl cellulose of the specific viscosity (as a 0.3 percent solution).

TABLE II  
Effect of methyl celluloses of different viscosities

| Viscosity type       | None  | Low   | Medium | High  | Extra high |
|----------------------|-------|-------|--------|-------|------------|
| Breaking length..... | 2,040 | 2,820 | 2,890  | 3,720 | 3,690      |
| Burst factor.....    | 15.5  | 24.1  | 25.2   | 34.0  | 35.3       |
| Tear factor.....     | 56.4  | 85.0  | 84.8   | 88.1  | 89.5       |

Using these figures, the following comparison may be calculated:

| Viscosity type       | None  | Average low and medium | Percent improvement over blank | Average high and extra high | Percent improvement over blank |
|----------------------|-------|------------------------|--------------------------------|-----------------------------|--------------------------------|
| Breaking length..... | 2,040 | 2,855                  | 40                             | 3,705                       | 82                             |
| Burst factor.....    | 15.5  | 24.65                  | 59                             | 34.65                       | 124                            |
| Tear factor.....     | 56.4  | 84.9                   | 51                             | 88.8                        | 57                             |

The proportion of treating material or its effective concentration in the beating liquor determines the physical characteristics of the paper sheets. This effect may be observed from the following summary of results.

TABLE III  
Effect of concentration of methyl cellulose

|                                                       |                      | Beating, hours. |       |       |       |
|-------------------------------------------------------|----------------------|-----------------|-------|-------|-------|
|                                                       |                      | 7               | 7     | 7     | 7     |
| Concentration, percent (based on weight of pulp)..... |                      | 0               | 1.2   | 6.0   | 12.0  |
| 10                                                    | Breaking length..... | 2,080           | 2,170 | 2,990 | 3,760 |
| Burst.....                                            |                      | 15.2            | 19.0  | 25.4  | 35.3  |

Thus, at a very low relative concentration of methyl cellulose, a decided improvement in mechanical properties is effected. At higher concentrations, the percentage increase in properties is correspondingly greater. The same amount of water was employed in each case, and the solution concentrations of methyl cellulose were 0.06, 0.3, and 0.6 percent.

15 The figure of the drawing is a graphic representation of the changes in tear factor, burst factor, and breaking length, in beating hull fiber pulp with 0.3 percent of methyl cellulose in the beater liquid (calculated at 6 percent on air-dry pulp) and without methyl cellulose.

20 Further, it has been found that the use of water-soluble methyl cellulose brings about a uniform increase in properties over a wide range of time intervals for beating, as will be noted from the figure. Both the curves in the figure and the data in Table V indicate that the improvements in paper qualities effected by methyl cellulose vary with the beating time. These qualities appear to develop at approximately corresponding times and in a somewhat similar manner and, in general, if a certain percentage of improvement is developed by beating in the presence of methyl cellulose, over a plain beating as a control, in a given short time, then a similar percentage of improvement is revealed in a longer time.

25 Further, it has been found that the beating liquor does not lose all of its methyl cellulose; but usually about 40 percent of the methyl cellulose is taken up by the fibers, while about 60 percent of that originally employed is carried forward in the white water discharged during the felting or sheet-forming operation. This white water can be immediately reused in the next beater run by introduction into the head box of the paper machine, preferably with an adjusting of the concentration of methyl cellulose therein. The paper product contains 0.1 to 6 percent of the cellulose ether distributed essentially uniformly throughout the mass of the article.

30 In connection with the acceleration in the production of beating effects by the present procedure, it may be pointed out that when pulp is undergoing beater action, it will at the start show low values of breaking length and burst factor. As the beating is continued, these values gradually increase, reach a maximum and then steadily decrease in volume. Measurement of the drainage time gives an indication of the change of these factors during beating. A standardized procedure exists for this measurement. When the pulp is underbeaten, the stock is free, shows a low drainage time and drains rapidly on the screens. When the pulp is overbeaten, it has a

35 high drainage time and drains very slowly; in this overbeaten condition, the pulp requires a slow-running paper-making machine and increased suction. A highly overbeaten stock is practically useless for general paper making because it drains too slowly and possesses poor paper

properties. It is found, in practice of this invention, that the drainage time increases slowly up to a point at which an optimum condition of the pulp is present, and thereupon a sudden increase of the drainage time occurs: when the pulp is withdrawn from beating at the time of this sudden jump, the burst factor and breaking length exhibit their optimum values. By way of example, in Table IV below, the drainage time up to about 8 hours of beating was 10 seconds or less: 10 while at 9 hours of beating, the drainage time had increased to 70 seconds, and further increase occurred later. In the experimental laboratory runs, a Valley type beater was used, with a pulp consistency between 4 and 5 percent. In a comparative test, it appeared that the experimental beater conditions were such that only half the beating time was required as compared with a commercial beater.

As a further example of practice, comparison operations were performed with bleached, second cut cotton linters, both in plain aqueous beating liquor and in a beating liquor containing methyl cellulose. In Table IV below are given the values obtained for a product when a medium viscosity methyl cellulose was employed at 12.0 percent concentration (based on weight of pulp, corresponding to 0.6 percent in the beater liquid), while in Table V the corresponding results are set out for the employment of 6.0 percent of high viscosity methyl cellulose, corresponding to 0.3 percent in the beater liquid.

TABLE IV  
Data on beating second cut linters

|                                                      | Beating, hours |       |       |       |
|------------------------------------------------------|----------------|-------|-------|-------|
|                                                      | 5              | 7     | 9     | 11    |
| Parts of methyl cellulose per 100 parts of pulp..... | 0              | 12.0  | 0     | 12.0  |
| Tear.....                                            | 75.7           | 90.0  | 53.6  | 105.0 |
| Breaking length.....                                 | 1,620          | 2,850 | 1,960 | 3,080 |
| Burst.....                                           | 13.1           | 23.3  | 15.0  | 29.0  |

TABLE V  
[Normal beating]

|                      | Beating, hours |       |       |       |       |
|----------------------|----------------|-------|-------|-------|-------|
|                      | 5              | 6     | 7     | 8     | 9     |
| Tear.....            | 61.5           | 56.4  | 56.4  | 49.0  | 46.8  |
| Breaking length..... | 1,550          | 1,920 | 2,040 | 2,160 | 2,190 |
| Burst.....           | 12.3           | 14.9  | 15.5  | 17.2  | 13.3  |

[With methyl cellulose]

|                                                         | Beating, hours |       |       |       |       |
|---------------------------------------------------------|----------------|-------|-------|-------|-------|
|                                                         | 5              | 6     | 7     | 8     | 9     |
| Methyl cellulose in liquor, percent.....                | 0.3            | 0.3   | 0.3   | 0.3   | 0.3   |
| Ratio methyl cellulose to pulp.....                     | 6.0            | 6.0   | 6.0   | 6.0   | 6.0   |
| Amount methyl cellulose on finished paper, percent..... | 1.64           | 88.8  | 2.67  | 2.74  | 3.03  |
| Tear.....                                               | 91.2           | 88.8  | 88.4  | 78.6  | 72.0  |
| Breaking length.....                                    | 2,720          | 3,290 | 3,700 | 3,890 | 4,220 |
| Burst factor.....                                       | 24.3           | 31.2  | 32.3  | 33.0  | 33.0  |

From Table IV, it will be noted that the average increase in properties obtained by beating the pulp in medium viscosity methyl cellulose solution, with four different beating times, corresponds to an increase in tear value of 104 percent,

in breaking length of 74 percent, and in burst value of 122 percent.

In Table V, the average increase in the test properties when 6.0 percent of high viscosity methyl cellulose was employed at five different beating times was found to be an increase of 55 percent in tear factor, 80 percent in breaking length, and 111 percent in burst value.

These results indicate the effectiveness of the employment of such material during a beating operation, and are particularly demonstrative of the efficiency of a high viscosity methyl cellulose. For example, although only half as much was used in Table V, as compared with that employed in Table IV, with medium viscosity methyl cellulose, yet the breaking length and burst values of the two pulps showed approximately the same average increment in the same beating time.

Tables IV and V are also indicative of the extent to which the beating time may be decreased by the presence of methyl cellulose. In Table IV, the breaking length, for example, reaches a value of 2030 at the end of 11 hours of beating in plain aqueous solution; while a value of 2850 is obtained by beating for 5 hours with methyl cellulose solution: thus, the beating time was decreased by more than 6 hours. In Table V, corresponding decreases are indicated.

When it is sought to employ this procedure with other agents in the beating liquor, care must be observed that these other agents are not incompatible with the action of the methyl cellulose, as such an effect tends to offset the value of the treating material. As a matter of comparison, the behavior of methyl cellulose in association with starch and paper-makers' alum was observed as follows:

TABLE VI  
Effect of starch and alum on methyl cellulose

|                                                                                                | Tear factor | Breaking length | Burst factor |
|------------------------------------------------------------------------------------------------|-------------|-----------------|--------------|
| Plain sulfite.....                                                                             | 120         | 2,230           | 17.2         |
| Sulfite plus methyl cellulose.....                                                             | 93          | 3,500           | 30.3         |
| Sulfite plus (starch and alum) at start; after beating 0.5 hours, add methyl cellulose.....    | 115         | 2,660           | 24.3         |
| Sulfite plus methyl cellulose at start; after beating 0.5 hours, add both starch and alum..... | 107         | 3,230           | 29.1         |

In each instance, the beating time was 1.5 hours, and the raw material was a bleached sulfite pulp. The concentration of methyl cellulose was 2 percent and where starch and alum were employed, a quantity of 2 percent of starch and 1 percent of alum was utilized. From this table, it will be noted that superior values are obtained by effecting the primary beating in the presence of methyl cellulose to obtain a proper fiber condition, prior to the introduction of starch, alum, or other agents. As a general rule of procedure, it is desirable that no material be introduced into the beating liquor prior to an initial action of the methyl cellulose or like agent upon the fibers, insofar as such added material may so modify the polar properties of the cellulose or of the liquor contents as a whole that adsorption of methyl cellulose on the fibers is diminished. The duration of beating prior to introduction of other furnish can be determined from the total beating time required for the desired reduction of the stock, and the time required for incorporating the other furnish, but must be sufficient for bringing the methyl cellulose to the individual fibers and for at least the initiation of fibrilla-

tion. A half hour has been found adequate in substantially all cases with a methyl cellulose solution, while an hour is practiced when the methyl cellulose is added in solid form, with commercial rates of beating.

In particular, it is pointed out that these effects are obtained without the employment of a subsequent heat treatment of such character as to melt and "set" the methyl cellulose, although heat may be advantageously employed to speed up the drying of the paper sheets, as in the usual commercial practice. The making of paper by the present procedure may therefore include the beating of aqueous suspension in the presence of cellulose ether, followed by the addition of sizing, etc., matters and the dilution of the pulp, the forming and draining of the sheets, and the drying and calendering operations.

As an indication of the increase in fold values as measured by the Schopper-tester, with different runs of treatment in which methyl cellulose was applied to a regular sulfite pulp furnish (after starch, size and alum had been introduced into the beater), it was found that foaming tended to occur; and hence it is further indicated to employ the preliminary beating with methyl cellulose before the other ingredients of the furnish are introduced. However, when the concentration of methyl cellulose is low (such as 0.2 percent), no serious foaming difficulty is to be noted, while the fold values of the product show definite improvement. The foam tends to carry methyl cellulose out of the beater, and hence to reduce the concentration apparently present.

The feasibility of obtaining extremely high fold values, or resistance to separation of fibers by repeated bending along a single line, is indicated by the following:

TABLE VII

| Percent methyl cellulose based on weight air-dry sulfite pulp | Percent methyl cellulose based on beater liquid | Percent improvement in fold value |
|---------------------------------------------------------------|-------------------------------------------------|-----------------------------------|
| 0.5                                                           | 0.025                                           | 90                                |
| 1.0                                                           | 0.050                                           | 200                               |
| 3.0                                                           | 0.150                                           | 370                               |
| 4.0                                                           | 0.200                                           | 660                               |
| 5.0                                                           | 0.250                                           | 1,470                             |

It has been found that methyl cellulose is an advantageous material for accomplishing the results sought, as its action begins at a very low concentration, and the effect becomes more pronounced with increasing concentrations.

It will be understood that ethyl and propyl celluloses may be similarly employed as the water-soluble cellulose ether, due attention being addressed to the lesser solubilities.

The effect has been obtained with cotton fibers including the cotton staple or lint, cotton linters, hull fiber, and manufactured cotton in which oxycellulose may have been formed; and also in sulfate, sulfite and soda pulps, in jute, manila hemp, and flax fibers. It thus is applicable generally to cellulosic fiber materials, including cotton fibers in raw condition or after subjection to chemical treatments, such as kier boiling or bleaching, in which the integrity of the fibers has been retained and they are in condition for fibrillation.

The exact behavior of the effective compounds in lowering the beating time is not entirely clear. However, it may be pointed out that two processes occur in the beater: one being the cutting action by which the lengths of the fibers are reduced, and the other being the fibrillation or the longitudinal splitting of the fibers. The latter action is obtained by beating a long time with very little pressure on the beater rolls, and is the preferred one because it gives a fine-bodied feltable stock with long fiber lengths. The action of methyl cellulose and like materials appears to be effective in decreasing the beating time and in improving the mechanical properties of the resulting paper product, by facilitating fibrillation (possibly by catalytic action) and in assuring a cementing of the fibrils during the sheet-forming operation.

It is obvious that the invention may be practiced in many ways other than those set out above, without departing from the scope of the appended claims.

We claim:

1. A sheet of beaten cotton fibers comprising the felted product of beating a fibrous cotton cellulosic material in aqueous suspension with a high viscosity water-soluble methyl cellulose, and characterized in containing at least substantially 2.4 percent of methyl cellulose and in having a tear factor in excess of 70, a breaking length in excess of 2500, and a burst strength in excess of 25.

2. The method of producing a sized feltable pulp from fibrous cellulosic materials, which includes the steps of beating the fibrous material in an aqueous suspension containing water-soluble methyl cellulose at least until fibrillation begins, thereafter adding a starch and alum sizing material, and continuing the beating operation until felting qualities are developed.

3. The method of producing sheets of felted fibrous cellulosic materials, which includes the step of beating the fibrous material in an aqueous solution whose solute essentially consists of substantially 0.3 percent methyl cellulose, with the solution present in the substantial quantity of 6.0 percent of water-soluble methyl cellulose by weight of air-dry pulp.

4. The method of producing strong sheets of fibrous cellulosic materials, which comprises beating the fibrous material in an aqueous solution whose solute consists essentially of water-soluble methyl cellulose in amount of 0.2 to 12 percent on the basis of air-dry pulp, and terminating the beating substantially coincident with a sudden increase of the drainage time of the material.

5. The method of producing paper sheets from fibrous cellulosic materials, which includes the steps of beating the fibrous materials in an aqueous solution whose solute consists essentially of 0.06 to 0.6 percent of water-soluble methyl cellulose of viscosity over 80 centipoises, until felting qualities are developed, and thereafter forming the sheet while retaining methyl cellulose therein.

DAVID M. MUSSER.  
HARRY C. ENGEL.